# EUROPEAN PATENT SPECIFICATION

(11) **EP 0 898 782 B1**
(45) Date of publication and mention of the grant of the patent: **09.07.2003**
(21) Application number: 97926529.5
(22) Date of filing: 14.05.1997
(51) Int. Cl.: H01J 29/88, H01J 29/06, H01J 31/12

(54) **FIELD EMISSION DISPLAYS WITH PRASEODYMIUM-MANGANESE OXIDE LAYER**
FELDEMISSIONSANZEIGEVORRICHTUNGEN MIT PRASEODYM-MANGAN-OXID-SCHICHT
SYSTEMES DE VISUALISATION A EMISSION PAR EFFET DE CHAMP AVEC COUCHE D'OXYDE DE PRASEODYME-MANGANESE

(30) Priority: 14.05.1996 US 645615; 31.12.1996 US 777797; 09.04.1997 US 840084
(43) Date of publication of application: 03.03.1999
(73) Proprietor: Micron Technology, Inc., Boise, ID 83706-0006 (US)
(72) Inventor: CHADHA, Surjit, S., Meridian, ID 83642 (US); RASMUSSEN, Robert, T., Boise, ID 83706 (US)
(74) Representative: Hoarton, Lloyd Douglas Charles
(86) International application number: US9708257
(87) International publication number: WO97043781

(56) References cited:
- DE-A- 19 526 042
- PATENT ABSTRACTS OF JAPAN vol. 013, no. 580 (P-980), 21 December 1989 & JP 01 244426 A (MATSUSHITA ELECTRIC IND CO LTD), 28 September 1989,
- PATENT ABSTRACTS OF JAPAN vol. 014, no. 538 (P-1136), 28 November 1990 & JP 02 230126 A (MATSUSHITA ELECTRIC IND CO LTD), 12 September 1990,
- PATENT ABSTRACTS OF JAPAN vol. 017, no. 157 (P-1511), 26 March 1993 & JP 04 322219 A (MATSUSHITA ELECTRIC IND CO LTD), 12 November 1992,
- NAOKI KAMEGASHIRA ET AL.: "thermochemical properties of PrMnO3 at high temperature" JOURNAL OF MATERIALS SCIENCE LETTERS, vol. 4, 1985, pages 103-104, XP002048642
- TOMIZO MATSUOKA ET AL.: "black Pr-Mn oxide dielectric material for AC thin-film electroluminescent display" J.ELECTROCHEM. SOC.:SOLID-STATE SCIENCE AND TECHNOLOGY, vol. 135, no. 7, July 1988, pages 1836-1839, XP002048866

## Description

This invention was made with Government support under Contract No. DABT63-93-C-0025 awarded by advanced Research Projects Agency (ARPA). The Government has certain rights in this invention.

### Technical Field

This invention relates generally to field emission displays and, more particularly, to a conductive, light-absorbing praseodymium-manganese oxide layer deposited on the surface of a baseplate within a field emission display to bleed off surface charge and absorb stray electrons.

### Background of the Invention

Many devices such as computers and televisions require the use of a display. Typically, the cathode ray tube (CRT) has been used to perform this function. The CRT consists of a scanning electron gun directed toward a phosphor-coated screen. The electron gun emits a stream of electrons that impinge upon individual phosphor picture elements or pixels on the screen. When the electrons strike the pixels, they cause the energy level of the phosphor to increase. As the energy level declines from this excited state, the pixels emit photons. These photons pass through the screen to be seen by a viewer as a point of light. The CRT, however, has a number of disadvantages. In order to scan the entire width of the screen, the CRT screen must be relatively distant from the electron gun. This makes the entire unit large and bulky. The CRT also requires a significant amount of power to operate.

More modem devices such as laptop computers require a light weight, portable screen. Currently, such screens use electroluminescent or liquid crystal display technology. A promising technology to replace these screens is the field emission display. The field emission display (FED) utilizes a baseplate of cold cathode emitter tips as a source of electrons in place of the scanning electron gun used in the CRT. When placed in an electric field, these emitter tips emit a stream of electrons in the direction of a faceplate to which phosphor pixels are adhered. Instead of a single gun firing electrons at the pixels, the FED has an array of emitter tips. Each of the emitter tips are individually addressable, and one or more of the emitter tips correspond to a single phosphor pixel on the faceplate.

One of the problems associated with an FED is that not all of the photons that are released from the pixels pass through the faceplate to be seen by the viewer as points of light. Rather, nearly half of the photons will proceed in the general direction of the baseplate, and may impinge upon the emitter tips and/or circuitry within the FED. This may cause an undesirable photoelectric effect, and any reflected light from the baseplate reduces the contrast of the FED. A further problem is that not all of the electrons released by the emitter tips actually excite their targeted pixel. Instead, some of these electrons are reflected internally, and may excite a non-targeted pixel.

Accordingly, there is a need in the art for a field emission display which minimizes the photoelectric effect, and the problems associated with internally-reflected electrons. The present invention fulfills these needs, and provides other related advantages.

### Summary of the Invention

In brief, this invention is generally directed to a conductive, light absorbing praseodymium-manganese oxide layer coated on the interior surface of an FED baseplate. The praseodymium-manganese oxide layer reduces the photoelectric effect and damage associated by reflected electrons from the faceplate, and improves display image and contrast due to absorption of any ambient light reaching the baseplate and/or by absorption of any photons emitted in the direction of the baseplate.

In one embodiment, a conductive and light-absorbing baseplate of a field emission display is disclosed. At least a portion of the interior surface of the baseplate (*i.e*., the surface opposite the faceplate) is coated with a praseodymium-manganese oxide layer having a resistivity which does not exceed 1 x 10⁵ Ω·cm, preferably does not exceed 1 x 10⁴ Ω·cm, and more preferably does not exceed 1 x 10³ Ω·cm. The praseodymium-manganese oxide layer is coated on the baseplate at a thickness ranging from 100 to 1500 nm (1,000Å to 15,000Å), and has a light absorption coefficient of at least 1 x 10⁵ cm⁻¹ at a wavelength of 500 nm.

In a related embodiment, an FED is disclosed which contains the conductive and light-absorbing baseplate of this invention. Such displays are particularly suited for use in products which are employed under high ambient light conditions, including (but not limited to) the screen of a laptop computer.

In a further embodiment, a process for manufacturing a conductive and light-absorbing baseplate is disclosed. The process includes coating the interior surface of the baseplate with a layer of praseodymium-manganese oxide having a resistivity which does not exceed 1 x 10⁵ Ω·cm. Suitable coating techniques include (but are not limited to) deposition by RF sputtering.

A process for manufacturing a conductive and light-absorbing praseodymium-manganese oxide material is disclosed. This process includes heating a mixture of a praseodymium compound and a manganese compound at a temperature ranging from 1200-1500°C for a period of time sufficient to yield the praseodymium-manganese oxide material. The praseodymium compound is Pr₆O₁₁ and the manganese compound is selected from MnO₂ and Mn(CO₃)₂. Furthermore, the ratio of praseodymium to manganese within the praseodymium-manganese oxide material is such that the material has a resistivity (after coating a layer of the same on the baseplate) that does not exceed 1 x 10⁵ Ω·cm.

These and other aspects of this invention will become evident upon reference to the attached figures and the following detailed description.

### Brief Description of the Drawings

Figure 1 is a cross-sectional view of a prior art field emission display screen, and illustrates both emitted and back-emitted photons, as well as internally-reflected electrons.
Figure 2 is a cross-sectional view of a representative field emission display of this invention.

### Detailed Description of the Invention

As mentioned above, the present invention is directed to a conductive, light absorbing praseodymium-manganese oxide layer for use within an FED. This layer serves to bleed off surface charge associated with stray electrons within the FED, and must have a resistivity no greater than 1x10⁵ Ω·cm, preferably no greater than 1x10⁴ Ω·cm, and more preferably no greater than 1x10³ Ω·cm. Furthermore, the praseodymium-manganese oxide layer also serves to absorb back-emitted photons (*i.e*., photons emitted from the faceplate in the direction of the baseplate). Due to its very dark color, the praseodymium-manganese oxide layer readily absorbs light (*i.e*., the light absorption coefficient of praseodymium-manganese oxide is on the order of 1x10⁵ cm⁻¹), which provides a number of benefits to the FED. One of these benefits is that it minimizes the photoelectric effect in the underlying circuitry due to stray photons striking the baseplate of the FED. A further beneficial property is that it provides better contrast between the emitted light and the ambient background reflection from the cathode surface.

The problems associated with existing FED screens is illustrated by reference to the prior art screen of Figure 1. Specifically, Figure 1 is a cross-sectional view of an FED screen 2 which is comprised of baseplate 3 and faceplate 4. Faceplate 4 includes an array of pixels 6 in contact with conductive layer 9, which in turn is in contact with a transparent material 5. Baseplate 3 includes an array of emitter tips 10 which protrude from a silicon substrate 12. A conductive layer 14 contacts the emitter tips to an addressing scheme (not shown) that selectively connects each of the emitter tips to a power supply (not shown). An insulating layer 16 surrounds each of the emitter tips 10. A conductive gate 18 also surrounds the emitter tips and is separated from conductive layer 14 and substrate 12 by insulating layer 16. Conductive grid 18 is connected to the positive terminal of a power supply through a similar addressing scheme (not shown) as that of the emitter tips. When a particular emitter tip is addressed, such as emitter tip 11 in Figure 1, an electric field is placed between the appropriate conductive gate and emitter tip. This electric field causes emitter tip 11 to release a stream of electrons (represented by arrows 17 and 19) toward pixel 7 located on faceplate 4.

For purpose of clarity, Figure 1 depicts a single pixel corresponding to each emitter tip. However, it should be recognized that more than one emitter tip may be associated with single pixel. Furthermore, the distance between faceplate 4 and baseplate 3 may be fixed by use of suitable supporting elements (not shown), and faceplate 4 and baseplate 3 are sealed along their edges and a high vacuum (e.g. 1.333 x 10⁻³ to 1.333 x 10⁻⁶Pa (1 x 10⁻⁵ to 1 x 10⁻⁸ torr)) is maintained therein.

When an electron (as depicted by arrow 19 of Figure 1) strikes phosphor pixel 7, the phosphor is elevated to an excited state and emits photon 8 as it drops back to a ground state. Photon 8 is seen by the viewer as a point of light. However, it is equally likely that the photon will be released back toward baseplate 3, as represented by photon 15. In this instance, photon 15 may create a photoelectric effect which leads to undesirable electrons and holes in the components of baseplate 3.

Figure 1 also illustrates a further problem associated with existing FED screens. Rather than exciting the phosphor pixel causing release of photons, electrons directed to a targeted pixel may be reflected, scattered or absorbed by the pixel. Some of these reflected electrons (as depicted by arrow 13 of Figure 1) and/or those produced by secondary emissions may travel back in the direction of baseplate 3, again resulting in unwanted electrons and producing holes in baseplate 3.

The present invention overcomes the above problems by employing a baseplate having a layer of praseodymium-manganese oxide upon the interior surface of the baseplate (*i.e*., the surface opposite the faceplate). As illustrated in Figure 2, an FED screen 20 of this invention contains faceplate 4 and baseplate 3. A praseodymium-manganese oxide layer 22 is in contact with conducting gate 18 which, in turn, is in contact with insulating layer 16 on conductive layer 14 and substrate 12. Emitter tips 10 and faceplate 4 (containing pixels 6, conductive layer 9 and transparent material 5) are the same as described above for Figure 1.

When a photon (as depicted by arrow 15 in Figure 2) strikes praseodymium-manganese oxide layer 22 it is absorbed, thus obviating the photoelectric effect and improving contrast of the FED. Electrons that are reflected back toward baseplate 3 (as depicted by arrow 13 in Figure 2) also impinge upon by the praseodymium-manganese oxide layer. Because the praseodymium-manganese oxide layer 22 is conductive, captured electrons are discharged through the conductivity gate 18 when the conductivity gate 18 is positively biased. Alternatively, if the praseodymium-manganese oxide layer 22 is electrically isolated from the conductivity gate 18, for example, by an intermediate insulative layer (not shown), the praseodymium-manganese oxide layer 22 could be grounded. In any event, the praseodymium-manganese oxide layer sharply reduces the number of electrons that impinge on components of baseplate 3, thus eliminating undesirable electron holes therein.

Accordingly, a praseodymium-manganese oxide material is disclosed which is used for depositing upon the interior surface of a baseplate of an FED. The praseodymium-manganese oxide material may be represented by the formula Pr:Mn:O₃, wherein the molar ratio of praseodymium to manganese (Pr:Mn) may generally range from 0.1:1 to 1:0.1, and preferably from 0.5:1 to 1:0.5. This molar ratio has been found to yield suitable conductivity for the resulting praseodymium-manganese oxide layer. Furthermore, by increasing the amount of manganese in relation to praseodymium, conductivity is increased (*i.e*., resistivity is decreased).

The praseodymium-manganese oxide material may be made by combining Pr₆O₁₁ with MnO₂ (or MnCO₃) in a mill jar, and milling the same to a powder containing particles having an average diameter of approximately 2 µm. This powder is then heated at a temperature ranging from 1200-1500°C, preferably from 1250-1430°C, for about 4 hours. After heating, the resulting material is very dark colored, essentially matte black. The heated material may then be re-crushed and milled to again yield a powder having an average particle diameter of about 2 µm.

As mentioned above, the ratio of Pr to Mn influences the conductivity of the resulting praseodymium-manganese oxide layer. Such a ratio may be controlled by the relative amounts of the components Pr₆O₁₁ and MnO₂ (or MnCO₃). Thus, these components are mixed in amounts sufficient to yield the Pr:Mn ratio disclosed above.

The praseodymium-manganese oxide material may be deposited on the interior surface of the baseplate by any number of techniques to a thickness ranging from 100 to 1500 nm (1,000Å to 15,000Å). Such deposition techniques are known to those skilled in this field, and include (but are not limited to) radio frequency (RF) sputtering, laser ablation, plasma deposition, chemical vapor deposition (CVD) and electron beam evaporation. For example, in the case of RF sputtering, the praseodymium-manganese oxide material is compressed to make a planar target, which is then mounted within a suitable backing plate for RF sputtering. Sputtering may then be carried out in an RF sputterer using argon or argon and oxygen gas, with a substrate temperature of 200-350°C and a sputtering pressure of about 0.799Pa (6 x 10⁻³ torr) to about 3.99Pa (3 x 10⁻² torr). With regard to CVD, organometallic precursors for Pr and Mn would be employed, such as Pr acetate, Pr oxalate or Pr(Thd)₃, as well as Mn acetate, Mn carbonyl, Mn methoxide and Mn oxalate.

The resistivity of the praseodymium-manganese oxide material may also be controlled by , for example, firing the material (after deposited as a layer on the interior surface of the baseplate) in a reducing atmosphere, such as hydrogen and/or carbon monoxide. Such treatment serves to increase conductivity (reducing resistivity) to levels suitable for use in the practice of this invention. Alternatively, additional components may be added to the material, such as conductive ions and/or metals, to further enhance conductivity.

The resulting praseodymium-manganese oxide layer on the interior surface of the baseplate shields the underlying circuitry from photons and stray electrons as discussed above. Since the praseodymium-manganese oxide layer is very dark colored, it also yields high contrast to the FED. Furthermore, an FED which employs the present invention possesses high legibility under ambient lighting conditions, and are particularly suited for use as screens for televisions, portable computers and as displays for outdoor use, such as avionics and automobiles.

The following examples are presented for purpose of illustration, not limitation.

### EXAMPLES

### Example 1

### Preparation of Praseodymium-Manganese Oxide Material

Pr₆O₁₁ and MnO₂ were purchased from a commercial source (Cerac, La Puente, CA) and used without further purification. Both components were placed in a mill jar (510.72 grams Pr₆O₁₁ and 86.94 grams MnO₂), 500 ml of isopropyl alcohol was added, and the resulting slurry milled for 24 hours at 100 rpm. The slurry was dried in an oven under a nitrogen atmosphere. The dried material was fired at 1350°C for 4 hours, and then cooled. The cooled material was ground to small particles (average diameter of about 2 µm) using a suitable grinding technique.

### Example 2

### Deposition of Praseodymium-Manganese Oxide Material on Baseplate

The resulting powdered material of Example 1 may be deposited on the baseplate by any of a variety of acceptable techniques. For example, in the case of RF sputtering, the powdered material may be sintered to form a planar sputter target. Sputtering may then be carried out in an RF sputterer using argon or argon and oxygen gas, with a substrate temperature of 200-350°C, and a pressure of about 0.799 Pa to 3.99 Pa (6x10⁻³ to 3x10⁻² torr).

### Example 3

### Manufacture of an FED Screen

The baseplate of Example 2 may used in the manufacture an FED screen using known techniques. The resulting FED has a number of advantages over existing products, including: reduced photoelectric effect; reduced damage by reflected electrons from the faceplate to the baseplate components; and improved display image and contrast due to absorption of any ambient light reaching the baseplate and/or by absorption of any photons emitted by the faceplate in the direction of the baseplate.

From the foregoing it will be appreciated that, although specific embodiments of this invention have been described herein for the purpose of illustration, various modifications may be made without deviating from the spirit and scope of this invention. Accordingly, this invention is not limited except as by the appended claims.

## Claims

1. A conductive and light-absorbing baseplate (3) of a field emission display, said baseplate (3) having an interior surface to the field emission display (20), wherein at least a portion of the interior surface is coated with a praseodymium-manganese oxide layer (22) having a resistivity which does not exceed 1 x 10⁵ Ωcm.

2. The baseplate (3) of Claim 1, wherein the praseodymium-manganese oxide layer (22) has a resistivity which does not exceed 1 x 10⁴ Ωcm.

3. The baseplate (3) of Claim 1, wherein the praseodymium-manganese oxide layer (22) has a resistivity which does not exceed 1 x 10³ Ωcm.

4. The baseplate (3) of Claim 1, wherein the praseodymium-manganese oxide layer (22) has a thickness which ranges from 100 to 1500 nm (1,000Å to 15,000Å).

5. The baseplate (3) of Claim 1, wherein the praseodymium-manganese oxide layer (22) has a light absorption coefficient of at least 1 x 10⁵ cm⁻¹ at a wavelength of 500 nm.

6. A field emission display (20) comprising a conductive and light-absorbing baseplate (3), wherein the baseplate (3) has an interior surface to the field emission display (20), and wherein at least a portion of the interior surface is coated with a praseodymium-manganese oxide layer (22) having a resistivity which does not exceed 1 x 10⁵ Ωcm.

7. The field emission display (20) of Claim 6, wherein the praseodymium-manganese oxide layer (22) has a resistivity which does not exceed 1 x 10⁴ Ωcm.

8. The field emission display (20) of Claim 6, wherein the praseodymium-manganese oxide layer (22) has a resistivity which does not exceed 1 x 10³ Ωcm.

9. The field emission display (20) of Claim 6, wherein the praseodymiummanganese oxide layer (22) has a thickness which ranges from 100 to 1500 nm (1,000Å to 15,000Å).

10. The field emission display (20) of Claim 6, wherein the praseodymium-manganese oxide layer (22) has a light absorption coefficient of at least 1 x 10⁵ cm⁻¹ at a wavelength of 500 nm.

11. A process for manufacturing a conductive and light-absorbing baseplate (3) of a field emission display (20), comprising coating at least a portion of the interior surface of the baseplate (3) with a layer (22) consisting essentially of praseodymium-manganese oxide, wherein the layer (22) has a resistivity which does not exceed 1 x 10⁵ Ωcm.

12. The process of Claim 11, wherein the layer (22) has a resistivity which does not exceed 1 x 10⁴ Ωcm.

13. The process of Claim 11, wherein the layer (22) has a resistivity which does not exceed 1 x 10³ Ωcm.

14. The process of Claim 11, wherein the layer (22) is coated to a thickness which ranges from 100 to 1500 nm (1,000Å to 15,000Å).

15. The process of Claim 11, wherein the layer (22) has a light absorption coefficient of at least 1 x 10⁵ cm⁻¹ at a wavelength of 500 nm.

16. The process of Claim 11, wherein the layer (22) is coated on the interior surface of the baseplate (3) by radiofrequency sputtering, laser ablation, plasma deposition, chemical vapor deposition or electron beam evaporation.

17. The process of Claim 11, wherein the layer (22) is coated on the interior surface of the baseplate (3) by radiofrequency sputtering.

18. The process of Claim 17, wherein Pr₆O₁₁ and a manganese source selected from MnO₂ and MnCO₃ form a sputtering target for the radiofrequency sputtering.

19. The process of Claim 11, wherein the layer (22) is coated on the interior surface of the baseplate (3) by chemical vapor deposition.

20. The process of Claim 19, wherein a praseodymium source selected from praseodymium acetate, praseodymium oxalate and Pr(Thd)₃ is used to form the layer (22).

21. The process of Claim 19, wherein a manganese source selected from manganese acetate, manganese carbonyl, manganese methoxide and manganese oxalate is used to form the layer (22).

22. The process of Claim 11 further comprising, after the coating step, the step of firing the layer (22) under a reducing atmosphere to lower its resistivity such that it does not exceed 1 x 10⁵ Ωcm.

23. The process of Claim 22, wherein the reducing atmosphere is formed of hydrogen, carbon monoxide or a mixture thereof.

24. The process of Claim 11, wherein the layer (22) further comprises a conductive ion.

25. The process of Claim 11, wherein the layer (22) further comprises a metal.

26. The process of Claim 11, wherein the layer (22) is formed of particles with an average particle diameter of 2 µm.

27. The process of Claim 11, wherein the layer (22) is in contact with a conducting gate (18).

28. The process of Claim 11, wherein the layer (22) is in contact with a insulative layer (16).

29. The process of Claim 11, wherein the layer (22) has a molar ratio of praseodymium-manganese ranging from 0.1:1 to 1:0.1.

30. The process of Claim 29, wherein the molar ratio ranges from 0.5:1 to 1:0.5.

31. The process of Claim 11, wherein the layer (22) comprises PrMnO₃.

32. The process of Claim 11 further comprising the step of assembling a field emission display (20) utilizing the conductive and light-absorbing baseplate (3).

33. A process for operating a field emission display (2) having a faceplate (4) and a baseplate (3), the process comprising absorbing photons with a layer (22) wherein at least a portion of the layer (22) consists essentially of praseodymium-manganese oxide, said layer (22) being disposed between the faceplate (4) and the baseplate (3) on the interior surface of the baseplate (3).

34. The process of Claim 33, wherein photons being emitted from the faceplate (4) in the direction of the baseplate (3) are absorbed.

35. The process of Claim 33, wherein the layer (22) has a resistivity which does not exceed 1 x 10⁵ Ωcm.

36. The process of Claim 33, wherein the layer (22) is a coating on the interior surface of the baseplate (3).

37. The process of Claim 36, wherein the layer (22) is coated on the interior surface of the baseplate (3) by radiofrequency sputtering, laser ablation, plasma deposition, chemical vapor deposition or electron beam evaporation.

38. The process of Claim 33, wherein the layer (22) further comprises a conductive ion.

39. The process of Claim 33, wherein the layer (22) further comprises a metal.

40. The process of Claim 33 wherein the layer (22) has a molar ratio of praseodymium-manganese ranging from 0.1:1 to 1:0.1.

41. The process of Claim 33, wherein the layer (22) comprises PrMnO₃.

42. The use of a layer (22) of praseodymium-manganese oxide having a resistivity which does not exceed 1 x 10⁵ Ωcm as a coating of at least a portion of a conductive and light-absorbing baseplate (3) of a field emission display (20).

43. The use of Claim 42, wherein the layer (22) has a resistivity which does not exceed 1 x 10⁴ Ωcm.

44. The use of Claim 42, wherein the layer (22) has a resistivity which does not exceed 1 x 10³ Ωcm.

45. The use of Claim 42 wherein the layer (22) is coated to a thickness which ranges from 100 to 1500 nm (1,000Å to 15,000Å).

46. The use of Claim 42, wherein the layer (22) has a light absorption coefficient of at least 1 x 10⁵ cm⁻¹ at a wavelength of 500 nm.

47. A process for manufacturing a conductive and light-absorbing praseodymium-manganese oxide coating on a baseplate (3) of a field emission display (20) comprising the steps of: heating a mixture of praseodymium compound and manganese compound to a temperature ranging from 1200-1500°C for a period of time sufficient to yield the praseodymium-manganese oxide coating material, wherein the molar ratio of the praseodymium compound to the manganese compound in the mixture prior to heating is such that the praseodymium-manganese oxide material has a resistivity that does not exceed 1 x 10⁵ Ωcm after the heating step, depositing the praseodymium-manganese oxide material on the interior surface of the baseplate.

48. The process of Claim 47 wherein the resistivity does not exceed 1 x 10⁴ Ωcm.

49. The process of Claim 47 wherein the resistivity does not exceed 1 x 10³ Ωcm.

50. The process of Claim 47 wherein, prior to the heating step, the mixture of the praseodymium compound and the manganese compound is milled to an average particle size of about 2 µm.

51. The process of Claim 47 wherein, after the heating step, the praseodymium-manganese oxide material is milled to an average particle size of about 2 µm.

52. The process of Claim 47 wherein the praseodymium compound is Pr₆O₄₉.

53. The process of Claim 47 wherein the manganese compound is MnO₂ or MnCO₃.

54. The process of Claim 47 wherein the molar ratio ranges from 0.1:1 to 1:0.1.

55. The process of Claim 47 wherein the molar ratio ranges from 0.5:1 to 1:0.5.

56. The process of Claim 47 wherein the praseodymium-manganese oxide material comprises PrMnO₃.

## Patentansprüche

1. Leitende und lichtabsorbierende Basisplatte (3) einer Feldemissionsanzeigevorrichtung, wobei die Basisplatte (3) eine Innenfläche an der Feldemissionsanzeigevorrichtung (20) aufweist und zumindest ein Abschnitt dieser Innenfläche mit einer Praseodym-Manganoxidschicht (22) beschichtet ist, deren spezifischer Widerstand 1 x 10⁵ Ωcm nicht übersteigt.

2. Basisplatte (3) nach Anspruch 1, wobei der spezifische Widerstand der Praseodym-Manganoxidschicht (22) 1 x 10⁴ Ωcm nicht übersteigt.

3. Basisplatte (3) nach Anspruch 1, wobei der spezifische Widerstand der Praseodym-Manganoxidschicht (22) 1 x 10³ Ωcm nicht übersteigt.

4. Basisplatte (3) nach Anspruch 1, wobei die Praseodym-Manganoxidschicht (22) eine Dicke im Bereich zwischen 100 und 1500 nm (1.000 Å bis 15.000 Å) aufweist.

5. Basisplatte (3) nach Anspruch 1, wobei die Praseodym-Manganoxidschicht (22) bei einer Wellenlänge von 500 nm einen Lichtabsorptionskoeffizient von mindestens 1 x 10⁵ cm⁻¹ aufweist.

6. Feldemissionsanzeigevorrichtung (20) mit einer leitenden und lichtabsorbierenden Basisplatte (3), wobei die Basisplatte (3) eine Innenfläche an der Feldemissionsanzeigevorrichtung (20) aufweist und wobei zumindest ein Abschnitt der Innenfläche mit einer Praseodym-Mangangoxidschicht (22) beschichtet ist, deren spezifischer Widerstand 1 x 10⁵ Ωcm nicht übersteigt.

7. Feldemissionsanzeigevorrichtung (20) nach Anspruch 6, wobei der spezifische Widerstand der Praseodym-Manganoxidschicht (22) 1 x 10⁴ Ωcm nicht übersteigt.

8. Feldemissionsanzeigevorrichtung (20) nach Anspruch 6, wobei der spezifische Widerstand der Praseodym-Mangangoxidschicht (22) 1 x 10³ Ωcm nicht übersteigt.

9. Feldemissionsanzeigevorrichtung (20) nach Anspruch 6, wobei die Praseodym-Manganoxid-schicht (22) eine Dicke zwischen 100 und 1500 nm (1000 Å und 15000 Å) aufweist.

10. Feldemissionsanzeigevorrichtung (20) nach Anspruch 6, wobei die Praseodym-Manganoxid-schicht (22) bei einer Wellenlänge von 500 nm einen Lichtabsorptionskoeffizienten von mindestens 1 x 10⁵ cm⁻¹ hat.

11. Verfahren zur Herstellung einer leitenden und lichtabsorbierenden Basisplatte (3) einer Feldemissionsanzeigevorrichtung (20), die das Beschichten zumindest eines Abschnitts der Innenfläche der Basisplatte (3) mit einer Schicht (22) umfaßt, die im wesentlichen aus Praseodym-Manganoxid besteht, wobei der spezifische Widerstand der Schicht 1 x 10⁵ Ωcm nicht übersteigt.

12. Verfahren nach Anspruch 11, wobei der spezifische Widerstand der Schicht 1 x 10⁴ Ωcm nicht übersteigt.

13. Verfahren nach Anspruch 11, wobei der spezifische Widerstand der Schicht 1 x 10³ Ωcm nicht übersteigt.

14. Verfahren nach Anspruch 11, wobei die Schicht (22) mit einer Dicke aufgetragen ist, die im Bereich zwischen 100 und 1500 nm (1000 Å und 15000 Å) liegt.

15. Verfahren nach Anspruch 11, wobei die Schicht (22) bei einer Wellenlänge von 500 nm einen Lichtabsorptionskoeffizienten von mindestens 1 x 10⁵ cm⁻¹ hat.

16. Verfahren nach Anspruch 11, wobei die Schicht (22) auf der Innenfläche der Basisplatte (3) durch Hochfrequenzbedampfen (RF-Sputtering), Laserabtragung, Plasmaabscheidung, chemische Dampfabscheidung oder Elektronenstrahlzerstäubung aufgetragen ist.

17. Verfahren nach Anspruch 11, wobei die Schicht (22) auf der Innenfläche der Basisplatte (3) durch Hochfrequenzbedampfen (RF-Sputtering) aufgetragen wird.

18. Verfahren nach Anspruch 17, wobei Pr₆O₁₁ und eine aus MnO₂ und MnCO₃ ausgewählte Manganquelle ein Bedampfungsziel des Hochfrequenzbedampfens bilden.

19. Verfahren nach Anspruch 11, wobei die Schicht (22) auf der Innenfläche der Basisplatte (3) durch chemische Dampfabscheidung aufgetragen wird.

20. Verfahren nach Anspruch 19, wobei eine aus Praseodymacetat, Praseodymoxalat und Pr(Thd)₃ ausgewählte Praseodymquelle dazu verwendet wird, die Schicht (22) zu bilden.

21. Verfahren nach Anspruch 19, wobei die aus Manganacetat, Mangankarbonyl, Manganmethoxid, und Manganoxalat gewählte Manganquelle dazu verwendet wird, die Schicht (22) zu bilden.

22. Verfahren nach Anspruch 11, das nach dem Schritt des Beschichtens den Schritt des Erhitzens der Schicht (22) in einer reduzierenden Atmosphäre umfaßt, um deren spezifischen Widerstand zu verringern, so daß dieser 1 x 10⁵ Ωcm nicht übersteigt.

23. Verfahren nach Anspruch 22, wobei die reduzierende Atmosphäre aus Wasserstoff, Kohlenmonoxid oder einer Mischung davon gebildet wird.

24. Verfahren nach Anspruch 11, wobei die Schicht (22) ferner ein leitendes Ion umfaßt.

25. Verfahren nach Anspruch 11, wobei die Schicht (22) ferner ein Metall umfaßt.

26. Verfahren nach Anspruch 11, wobei die Schicht (22) aus Partikeln mit einem durchschnittlichen Partikeldurchmesser von 2 µm gebildet ist.

27. Verfahren nach Anspruch 11, wobei die Schicht (22) in Kontakt mit einem leitenden Gitter (18) ist.

28. Verfahren nach Anspruch 11, wobei die Schicht (22) in Kontakt mit einer isolierenden Schicht (16) ist.

29. Verfahren nach Anspruch 11, wobei die Schicht (22) ein molares Verhältnis von Praseodym und Mangan zwischen 0,1 : 1 und 1 : 0,1 hat.

30. Verfahren nach Anspruch 29, wobei das molare Verhältnis zwischen 0,5 : 1 und 1 : 0,5 liegt.

31. Verfahren nach Anspruch 11, wobei die Schicht (22) PrMnO₃ umfaßt.

32. Verfahren nach Anspruch 11, das ferner den Schritt des Zusammensetzens einer Feldemissionsanzeigevorrichtung (20) umfaßt, wobei die leitende und lichtabsorbierende Basisplatte (3) verwendet wird.

33. Verfahren zum Betreiben einer Feldemissionsanzeige (2) mit einer Frontplatte (4) und einer Basisplatte (3), wobei das Verfahren ein Absorbieren von Photonen mittels einer Schicht (22) umfaßt, von der zumindest ein Abschnitt im wesentlichen aus Praseodym-Manganoxid besteht und wobei die Schicht (22) zwischen der Frontplatte (4) und der Basisplatte (3) auf der Innenfläche der Basisplatte (3) aufgebracht ist.

34. Verfahren nach Anspruch 33, wobei die von der Frontplatte (4) in Richtung der Basisplatte (3) emittierten Photonen absorbiert werden.

35. Verfahren nach Anspruch 33, wobei der spezifische Widerstand der Schicht (22) 1 x 10⁵ Ωcm nicht übersteigt.

36. Verfahren nach Anspruch 33, wobei die Schicht (22) eine Beschichtung auf der Innenfläche der Basisplatte (3) ist.

37. Verfahren nach Anspruch (36), wobei die Schicht (22) auf der Innenfläche der Basisplatte (3) durch Hochfrequenzbedampfen (RF-Sputtering), Laserabtragung, Plasmaabscheidung, chemische Dampfabscheidung oder Elektronenstrahlzerstäubung aufgetragen ist.

38. Verfahren nach Anspruch 33, wobei die Schicht (22) ferner ein leitendes Ion umfaßt.

39. Verfahren nach Anspruch 33, wobei die Schicht (22) ferner ein Metall umfaßt.

40. Verfahren nach Anspruch 33, wobei die Schicht (22) ein Molverhältnis von Praseodym zu Mangan zwischen 0,1 : 1 und 1 : 0,1 aufweist.

41. Verfahren nach Anspruch 33, wobei die Schicht (22) PrMnO₃ umfaßt.

42. Verwendung einer Schicht (22) aus Praseodym-Manganoxid, deren spezifischer Widerstand 1 x 10⁵ Ωcm nicht übersteigt, als Beschichtung zumindest eines Abschnittes einer leitenden und lichtabsorbierenden Basisplatte (3) einer Feldemissionsanzeigevorrichtung (20).

43. Verwendung nach Anspruch 42, wobei der spezifische Widerstand der Schicht (22) 1 x 10⁴ Ωcm nicht übersteigt.

44. Verwendung nach Anspruch 42, wobei der spezifische Widerstand der Schicht (22) 1 x 10³ Ωcm nicht übersteigt.

45. Verwendung nach Anspruch 42, wobei die Schicht (22) mit einer Dicke zwischen 100 und 1500 nm (1000 Å und 15000 Å) aufgetragen ist.

46. Verwendung nach Anspruch 42, wobei die Schicht (22) bei einer Wellenlänge von 500 nm einen Lichtabsorptionskoeffizienten von mindestens 1 x 10⁵ cm⁻¹ hat.

47. Verfahren zur Herstellung einer leitenden und lichtabsorbierenden Praseodym-Manganoxidbeschichtung auf einer Basisplatte (3) einer Feldemissionsanzeigevorrichtung (20), das die Schritte umfaßt: Erhitzen eines Gemischs aus einer Praseodymverbindung und einer Manganverbindung auf eine Temperatur zwischen 1200°C und 1500°C für eine Zeitperiode, die ausreicht, das Praseodym-Manganoxidbeschichtungsmaterial zu erhalten, wobei das molare Verhältnis der Praseodymverbindung und der Manganverbindung in dem Gemisch vor dem Erhitzen so ist, daß das Praseodym-Manganoxidmaterial einen spezifischen Widerstand hat, der nach dem Schritt des Erhitzens 1 x 10⁵ Ωcm nicht übersteigt, und Ablagern des Praseodym-Manganoxidmaterials auf der Innenfläche der Basisplatte.

48. Verfahren nach Anspruch 47, wobei der spezifische Widerstand 1 x 10⁴ Ωcm nicht übersteigt.

49. Verfahren nach Anspruch 47, wobei der spezifische Widerstand 1 x 10³ Ωcm nicht übersteigt.

50. Verfahren nach Anspruch 47, wobei vor dem Schritt des Erhitzens das Gemisch aus der Praseodymverbindung und der Manganverbindung auf eine durchschnittliche Partikelgröße von ungefähr 2 um gemahlen wird.

51. Verfahren nach Anspruch 47, wobei nach dem Schritt des Erhitzens das Praseodym-Manganoxidmaterial auf eine durchschnittliche Partikelgröße von ungefähr 2 µm gemahlen wird.

52. Verfahren nach Anspruch 47, wobei die Praseodymverbindung Pr₆O₄₉ ist.

53. Verfahren nach Anspruch 47, wobei die Manganverbindung MnO₂ oder MnCO₃ ist.

54. Verfahren nach Anspruch 47, wobei das molare Verhältnis zwischen 0,1 : 1 und 1 : 0,1 liegt.

55. Verfahren nach Anspruch 47, wobei das molare Verhältnis zwischen 0,5 : 1 und 1 : 0,5 liegt.

56. Verfahren nach Anspruch 47, wobei das Praseodym-Manganoxidmaterial PrMnO₃ umfaßt.

## Revendications

1. Une plaque de base photo-absorbante et conductrice (3) d'un afficheur à émission par effet de champ, ladite plaque de base (3) ayant une surface intérieure à l'afficheur à émission par effet de champ (20), dans laquelle au moins une partie de la surface intérieure est recouverte d'une couche d'oxyde de praséodyme-manganèse (22) ayant une résistivité qui n'excède pas 1 x 10⁵ Ωcm.

2. La plaque de base (3) de la Revendication 1, dans laquelle la couche d'oxyde de praséodyme-manganèse (22) a une résistivité qui n'excède pas 1 x 10⁴ Ωcm.

3. La plaque de base (3) de la Revendication 1, dans laquelle la couche d'oxyde de praséodyme-manganèse (22) a une résistivité qui n'excède pas 1 x 10³ Ωcm.

4. La plaque de base (3) de la Revendication 1, dans laquelle la couche d'oxyde de praséodyme-manganèse (22) a une épaisseur qui est comprise entre 100 et 1500 nm (1.000 Å et 15.000 Å).

5. La plaque de base (3) de la Revendication 1, dans laquelle la couche d'oxyde de praséodyme-manganèse (22) a un coefficient de photo-absorption d'au moins 1 x 10⁵ cm⁻¹ à une longueur d'onde de 500 nm.

6. Un afficheur à émission par effet de champ (20) comprenant une plaque de base photo-absorbante et conductrice (3), dans lequel la plaque de base a une surface intérieure à l'afficheur à émission par effet de champ (20), et dans lequel au moins une partie de la surface intérieure est recouverte d'une couche d'oxyde de praséodyme-manganèse (22) ayant une résistivité qui n'excède pas 1 x 10⁵ Ωcm.

7. L'afficheur à émission par effet de champ (20) de la Revendication 6, dans lequel la couche d'oxyde de praséodyme-manganèse (22) a une résistivité qui n'excède pas 1 x 10⁴ Ωcm.

8. L'afficheur à émission par effet de champ (20) de la Revendication 6, dans lequel la couche d'oxyde de praséodyme-manganèse (22) a une résistivité qui n'excède pas 1 x 10³ Ωcm.

9. L'afficheur à émission par effet de champ (20) de la Revendication 6, dans lequel la couche d'oxyde de praséodyme-manganèse (22) a une épaisseur qui est comprise entre 100 et 1500 nm (1.000 Å et 15.000 Å).

10. L'afficheur à émission par effet de champ (20) de la Revendication 6, dans lequel la couche d'oxyde de praséodyme-manganèse (22) a un coefficient de photo-absorption d'au moins 1 x 10⁵ cm⁻¹ à une longueur d'onde de 500 nm.

11. Un procédé pour fabriquer une plaque de base photo-absorbante et conductrice (3) d'un afficheur à émission par effet de champ (20), comprenant la couverture d'au moins une partie de la surface intérieure de la plaque de base (3) avec une couche (22) consistant essentiellement en oxyde de praséodyme-manganèse, selon lequel la couche (22) a une résistivité qui n'excède pas 1 x 10⁵ Ωcm.

12. Le procédé de la Revendication 11, selon lequel la couche (22) a une résistivité qui n'excède pas 1 x 10⁴ Ωcm.

13. Le procédé de la Revendication 11, selon lequel la couche (22) a une résistivité qui n'excède pas 1 x 10³ Ωcm.

14. Le procédé de la Revendication 11, selon lequel la couché (22) est recouverte d'une épaisseur qui est comprise entre 100 et 1500 nm (1.000 Å et 15.000Å).

15. Le procédé de la Revendication 11, selon lequel la couche (22) a un coefficient de photo-absorption d'au moins 1 x 10⁵ cm⁻¹ à une longueur d'onde de 500 nm.

16. Le procédé de la Revendication 11, selon lequel la couche (22) est recouverte sur la surface intérieure de la plaque de base (3) par pulvérisation à radiofréquence, ablation par laser, dépôt par plasma, dépôt chimique en phase vapeur ou évaporation par faisceau d'électrons.

17. Le procédé de la Revendication 11, selon lequel la couche (22) est recouverte sur la surface intérieure de la plaque de base (3) par pulvérisation à radiofréquence.

18. Le procédé de la Revendication 17, selon lequel Pr₆O₁₁ et une source de manganèse sélectionnée parmi du MnO₂ et MnCO₃ forment une cible de pulvérisation pour la pulvérisation à radiofréquence.

19. Le procédé de la Revendication 11, selon lequel la couche (22) est recouverte sur la surface intérieure de la plaque de base (3) par dépôt chimique en phase vapeur.

20. Le procédé de la Revendication 19, selon lequel une source de praséodyme sélectionnée parmi l'acétate de praséodyme, l'oxalate de praséodyme et Pr(Thd)₃ est utilisée pour former la couche (22).

21. Le procédé de la Revendication 19, selon lequel une source de manganèse sélectionnée à partir d'acétate de manganèse, de carbonylique de manganèse, de méthoxide de manganèse et d'oxalate de manganèse est utilisée pour former la couche (22).

22. Le procédé de la Revendication 11 comprenant en outre, après l'étape de recouvrement, l'étape de chauffe de la couche (22) sous une atmosphère de réduction pour abaisser sa résistivité de sorte qu'elle n'excède pas 1 x 10⁵ Ωcm.

23. Le procédé de la Revendication 22, dans lequel l'atmosphère de réduction est formé d'hydrogène, de monoxyde de carbone ou d'un mélange de ceux-ci.

24. Le procédé de la Revendication 11, dans lequel la couche (22) comprend en outre un ion conducteur.

25. Le procédé de la Revendication 11, dans lequel la couche (22) comprend en outre un métal.

26. Le procédé de la Revendication 11, selon lequel la couche (22) est formée de particules avec un diamètre de particule moyen de 2 µm.

27. Le procédé de la Revendication 11, selon lequel la couche (22) est en contact avec une grille conductrice (18).

28. Le procédé de la Revendication 11, selon lequel la couche (22) est en contact avec une couche isolante (16).

29. Le procédé de la Revendication 11, selon lequel la couche (22) a un rapport moléculaire de praséodyme-manganèse compris entre 0,1:1 et 1:0,1.

30. Le procédé de la Revendication 29, dans lequel le rapport moléculaire est compris entre 0,5:1 et 1:0,5.

31. Le procédé de la Revendication 11, dans lequel la couche (22) comprend du PrMnO₃.

32. Le procédé de la Revendication 11, comprenant en outre l'étape d'assembler un afficheur par effet de champ (20) utilisant la plaque de base photo-absorbante et conductrice (3).

33. Un procédé pour faire fonctionner un afficheur par effet de champ (2) ayant une plaque avant (4) et une plaque de base (3), le procédé comprenant l'absorption de photons avec une couche (22), selon lequel au moins une partie de la couche (22) consiste essentiellement en oxyde de praséodyme-manganèse, ladite couche (22) étant disposée entre la plaque avant (4) et la plaque de base (3) sur la surface intérieure de la plaque de base (3).

34. Le procédé de la Revendication 33, selon lequel des photons émis à partir de la plaque avant (4) dans la direction de la plaque de base (3) sont absorbés.

35. Le procédé de la Revendication 33, selon lequel la couche (22) a une résistivité qui n'excède pas 1 x 10⁵ Ωcm.

36. Le procédé de la Revendication 33, selon lequel la couche (22) est une couverture de la surface intérieure de la plaque de base (3).

37. Le procédé de la Revendication 36, selon lequel la couche (22) est recouverte sur la surface intérieure de la plaque de base (3) par pulvérisation à radiofréquence, ablation par laser, dépôt par plasma, dépôt chimique en phase vapeur ou évaporation par faisceau d'électrons.

38. Le procédé de la Revendication 33, selon lequel la couche (22) comprend en outre un ion conducteur.

39. Le procédé de la Revendication 33, selon lequel la couche (22) comprend en outre un métal.

40. Le procédé de la Revendication 33, selon lequel la couche (22) a un rapport moléculaire de praséodyme-manganèse s'étendant de 0,1:1 à 1:0,1.

41. Le procédé de la Revendication 33, selon lequel la couche (22) comprend du PrMnO₃.

42. L'utilisation d'une couche (22) d'oxyde de praséodyme-manganèse ayant une résistivité qui n'excède pas 1 x 10⁵ Ωcm en tant que recouvrement d'au moins une partie d'une plaque de base photo-absorbante et conductrice (3) d'un afficheur à émission par effet de champ (20).

43. L'utilisation de la Revendication 42, dans lequel la couche (22) a une résistivité qui n'excède pas 1 x 10⁴ Ωcm.

44. L'utilisation de la Revendication 42, dans lequel la couche (22) a une résistivité qui n'excède pas 1 x 10³ Ωcm.

45. L'utilisation de la Revendication 42, dans lequel la couche (22) est recouverte d'une épaisseur qui est comprise entre 100 et 1500 nm (1.000Å et 15.000Å).

46. L'utilisation de la Revendication 42, dans lequel la couche (22) a un coefficient de photo-absorption d'au moins 1 x 10⁵ cm⁻¹ à une longueur d'onde de 500 nm.

47. Un procédé pour fabriquer un recouvrement d'oxyde de praséodyme-manganèse photo-absorbante et conductrice sur une plaque de base (3) d'un afficheur à émission par effet de champ (20) comprenant les étapes de : chauffer un mélange de composé de praséodyme et de composé de manganèse à une température de 1200-1500°C pour une période de temps suffisante pour produire le matériau de recouvrement d'oxyde de praséodyme-manganèse, selon lequel le rapport moléculaire du composé praséodyme au composé manganèse dans le mélange préalablement à la chauffe est tel que le matériau d'oxyde de praséodyme-manganèse a une résistivité qui n'excède pas 1 x 10⁵ Ωcm après l'étape de chauffe, déposer le matériau d'oxyde de praséodyme-manganèse sur la surface intérieure de la plaque de base.

48. Le procédé de la Revendication 47 selon lequel la résistivité n'excède pas 1 x 10⁴ Ωcm.

49. Le procédé de la Revendication 47 selon lequel la résistivité n'excède pas 1 x 10³ Ωcm.

50. Le procédé de la Revendication 47 selon lequel, préalablement à l'étape de chauffe, le mélange du composé de praséodyme et du composé de manganèse est fraisé à une dimension particulaire moyenne d'environ 2 µm.

51. Le procédé de la Revendication 47 selon lequel, après l'étape de chauffage, le matériel d'oxyde de praséodyme-manganèse est broyé en une taille de particule moyenne d'environ 2 µm.

52. Le procédé de la Revendication 47 selon lequel le composé de praséodyme est Pr₆O₄₉.

53. Le procédé de la Revendication 47 selon lequel le composé de manganèse est MnO₂ ou MnCO₃.

54. Le procédé de la Revendication 47 selon lequel le rapport moléculaire est compris entre 0,1:1 et 1:0,1.

55. Le procédé de la Revendication 47 selon lequel le rapport moléculaire est compris entre 0,5:1 et 1:0,5.

56. Le procédé de la Revendication 47 selon lequel le matériau d'oxyde de praséodyme-manganèse comprend PrMnO₃.
